

## UNITED STATES PATENT OFFICE

2,221,319

## MAGNESIUM BASE ALLOY

Hubert Altwicker, Bitterfeld, and Wilhelm Rosenkranz, Sandersdorf, near Bitterfeld, Germany, assignors, by mesne assignments, to Magnesium Development Corporation, a corporation of Delaware

No Drawing. Application October 22, 1938, Serial No. 236,574. In Germany November 22, 1937

3 Claims. (Cl. 75—168)

This invention relates to magnesium alloys. The high percentage magnesium alloys usually employed, for plastic deformation, are known to fall into two groups. The alloys of one of these groups contain a comparatively substantial proportion of alloying components, especially aluminium (e. g. between 6 and 10%) if desired, together with zinc (between 0.5 and 1%), and consequently have in the deformed condition, a considerable tensile strength (e. g. between 28 and 37 kgs. per sq. mm.) and high yield point (e. g. between 20 and 28 kgs. per sq. mm.) with good elongation (e. g. between 7 and 16%) (see text book on "Magnesium alloys with special reference to Elektron" 2nd edition 1934, sheet 13, alloys AZM and AZ 855). These alloys, however, have the disadvantage of being somewhat difficult to work by plastic deformation, even in the warm state. The magnesium alloys of the other of the two above referred to groups contain a comparatively small proportion only of alloying components, and this latter group is almost exclusively represented by alloys in which, in addition to magnesium, and apart from the usual impurities only manganese is present in amounts up to about 2.5% and preferably about 2.0% (loc. cit., alloy AM 503). Alloys of this latter group are distinguished by high resistance to corrosion, good welding properties and excellent malleability in the warm, but, owing to the absence of the known hardening components aluminium and zinc, they possess a relatively low tensile strength (e. g. between 19 and 25 kgs. per sq. mm.), low yield point (e. g. between 14 and 17 kgs. per sq. mm.) and small elongation (e. g. between 1.5 and 5%).

As the result of endeavours to combine the advantages of both groups of alloys, viz. high tensile strength, yield point and elongation and resistance to corrosion, it has now been ascertained that it is possible to impart to the alloys of the second group, which contain as alloying constituents substantially only manganese in amounts up to about 2.5%, properties which meet the foregoing requirements, by the addition of small amounts of cerium, or other rare earth elements, up to about 1%. Such addition improves the strength, yield point and elongation of the plastically deformed alloys of magnesium and manganese to such an extent that the values for the constants become at least equal to those of the alloys of said first mentioned group, whilst the welding properties, resistance to corrosion, and malleability, are not rendered inferior to the binary magnesium-manganese alloys. The malleability, in the cold state, is even improved by comparison with the alloys of the last named group, so that it is possible, for example to work up the new alloys in the cold into sheets, without difficulty.

The physical properties of the aforesaid alloys may be further improved by an addition of aluminium and/or zinc in a total quantity of up to about 1% without impairing other favourable properties of the alloys. When adding zinc in this manner, the mechanical properties are generally improved; small quantities of aluminium ranging between about 0.1 and 0.5%, on the other hand, result in an improvement of the capability of the alloys for plastic deformation, such as extruding, forging, and rolling, and thus enable to produce thinner sections at comparatively low temperatures of deformation. In these latter alloys the elongation is lowered but slightly, whilst particularly the yield point, and to some extent also the tensile strength of the products, is substantially increased.

The following representative examples show the improved physical properties of the alloys according to the invention as compared with pure magnesium or with magnesium containing corresponding quantities of either cerium or manganese singly.

## 1. MATERIAL PRESSED INTO RODS AT 360° C.

| No. | Alloy                                       | Mechanical properties              |                     |                               |
|-----|---------------------------------------------|------------------------------------|---------------------|-------------------------------|
|     |                                             | Tensile strength, kgs. per sq. mm. | Elongation, percent | Yield point, kgs. per sq. mm. |
| 1   | Pure magnesium                              | 17.0                               | 8.0                 | 10.0                          |
| 2   | Pure magnesium with 1.0% Ce                 | 19.8                               | 23.2                | 10.7                          |
| 3   | Pure magnesium with 2% Mn                   | 22.0                               | 2.0                 | 15.0                          |
| 4   | Pure magnesium with 2% Mn, 0.4% Ce          | 28.7                               | 8.4                 | 24.8                          |
| 5   | Pure magnesium with 2% Mn, 0.7% Ce          | 26.5                               | 11.0                | 22.1                          |
| 6   | Pure magnesium with 2% Mn, 0.4% Ce, 0.6% Zn | 31.9                               | 7.0                 | 23.3                          |

## 2. MATERIAL ROLLED INTO SHEETS 1 MM. THICK AT 460 TO 420° C.

|   |                                    |       |       |       |
|---|------------------------------------|-------|-------|-------|
| 7 | Pure magnesium with 2% Mn          | 19.0  | 5.0   | 8.0   |
| 8 | Pure magnesium with 2% Mn, 0.4% Ce | 26-28 | 16-25 | 19-24 |

The term "yield point" used herein is intended to denote the load in kilogrammes per square millimetre applied to a test bar which will produce a permanent elongation of 0.2% on a measured length of test bar.

The alloys of the present invention are especially suitable for wrought goods, e. g. sheets, extrusions and forgings. The maximum permissible cerium content can be regarded as 1.5%, but 5 preferably not more than about 1% is to be used.

The cerium in the alloys according to the invention may be replaced by the so-called "cerium Mischmetall," and in the appended claims the 10 term "cerium" is to be construed as also including the latter mixture of metals.

We claim:

1. An alloy containing between about 0.1 and about 2.5% of manganese, between about 0.1 and 15 about 1% of cerium, and between about 0.1 and about 1% of zinc, the balance being magnesium.

2. An alloy containing between about 0.1 and about 2.5% of manganese, between about 0.1 and about 1% of cerium, and between about 0.1 and 0.5% of aluminium, the balance being magnesium.

3. A magnesium base alloy containing between about 0.1 and about 1.5% of cerium and between about 0.1 and about 2.5% of manganese, characterized by improved tensile strength, yield strength, ductility, and workability in both hot 10 and cold conditions with respect to the same alloy devoid of cerium.

HUBERT ALTWICKER.  
WILHELM ROSENKRANZ. 15